

Oct. 6, 1931.

M. S. McCONOUGHY

1,826,217

LINOLEUM PRODUCT AND METHOD OF MAKING SAME

Filed Sept. 10, 1927



Fig. 1.



Fig. 2.



Fig. 3.



Fig. 4.



Fig. 5.



Fig. 6.

INVENTOR

MERLE S. MC CONOUGHY

BY Gordon C. Willard

ATTORNEY

## UNITED STATES PATENT OFFICE

MERLE S. MC CONOUGHEY, OF EAST ORANGE, NEW JERSEY, ASSIGNOR TO CONGOLEUM-NAIRN, INC., A CORPORATION OF NEW YORK

## LINOLEUM PRODUCT AND METHOD OF MAKING SAME

Application filed September 10, 1927. Serial No. 213,606.

My present invention concerns the final commercial product known as linoleum and commonly used as a floor covering, rather than the special compositions or cements 5 from which this product may be made.

Various primary types of the floor coverings that are called linoleum were invented and were named "linoleum" by Walton more than fifty years ago. His original linoleum 10 compositions included oxidized (polymerized) linseed oil, resin and kauri gum specially prepared and combined with pigments, wood pulp, ground cork or similar filling material. It is characteristic of these compositions 15 that they are plastic when hot so that they can be easily rolled to sheet form; that they will set sufficiently for handling when cooled and that thereafter they can be further cured and oxidized to the elastic firmness, characteristic of the finished products, 20 by long continued exposure to hot air. Walton also invented various methods whereby such compositions are rolled or cemented in sheet form on a fabric backing of jute or the 25 like, and the backing was customarily painted, thereby improving the appearance of the under surface of the linoleum and affording some protection against abrasion and moisture.

While many changes have since been made 30 in the proportions of the materials used in the linoleum compositions and various additions and substitutions have been made, sometimes with a view to decreasing the proportion 35 of the linseed oil and other costly constituents and sometimes with a view to improving some quality of the product, the essential constituents of the linoleum compositions and also the structure and physical 40 characteristics of the completed product are to-day generically the same as they were fifty years ago.

This product has been and is a great commercial success on account of its well known 45 virtues, and notwithstanding several equally well known weaknesses and defects. I have discovered that though these defects and weaknesses are quite different in kind, it is a remarkable fact that they all happen to be 50 eliminated or substantially remedied by dif-

ferently directed aspects, or functionings of a novel fabric employed in accordance with my present invention. Among these weaknesses and defects may be mentioned the following:

First: It has always been found difficult to sheet the linoleum composition onto the fabric so that the product will remain uniformly flat, particularly where the fabric is the preferred jute burlap, because this fabric 55 is of very loose, slippery, open weave and is also non-uniform as to sizes and degree of twist in the threads or yarns from which it is woven. Moreover, even the best linoleums of the present day art exhibit strong tendency 60 to warp, convex, and billow when the back or painted face is laid next to the floor where it can sweat and become moist in various ways. As the result, it long ago came to be accepted that a linoleum floor covering should 65 be cemented to the floor. But this is not satisfactory because it is difficult and expensive to get a cement sufficiently adhesive and waterproof to hold the linoleum against convexing or "blistering", as it is called, under 70 trying conditions which are sure to arise sooner or later even in the best regulated installations. Furthermore, this defect prevents the extensive use of linoleum in the 75 form of rugs, which, of course, cannot be 80 cemented at all.

It has long been recognized that moisture getting under the linoleum is the cause of this blistering or billowing, and the history of the art shows that experts have long sought to 85 keep the water out by waterproofing the under surface of the linoleum, typical remedies including protective coatings of waterproofing paint, linoleum composition, rubber solution, asphalt, etc., painted, rolled or otherwise applied to the under or floor surface of the linoleum. It has also been proposed to use asphalt saturated felt as the floor face of the linoleum, but all of these expedients have 90 proved commercial failures for one reason or another. No one has ever succeeded in getting a coating of paint, rubber or asphalt that is sufficiently waterproof to prevent convexing under conditions of practical use on 95 the floor, while the attempts to hold down the 100

linoleum by using asphalt saturated felt, etc., for the back or floor face of the linoleum have resulted in a product lacking in many of the desirable qualities which the trade expects and demands when it buys linoleum.

By my invention I am able to preserve the physical structure, appearance, and the qualities now associated with the name linoleum, while at the same time completely eliminating all tendency of the linoleum to warp or convex when in use. At the same time I take care of the second, entirely different set of defects which may be briefly described as follows:

15 Second: The open-mesh, basket weave fabrics most suitable for properly interlocking with and "anchoring" the linoleum composition, are difficult to handle in the automatic machinery for rolling or cementing on 20 the linoleum composition and heretofore starch, starch sizing, paint and other fillers have been used to stiffen the burlap. In the finished product the starch, paint and other filling materials tend to become rigid and 25 brittle with time, constituting a thin layer, interpenetrating with rigid mortar like bonds, the fibers of the burlap. Hence, when flat linoleum is rolled or warped linoleum flattened, these rigid bonds tend to tear loose 30 and the brittle layer breaks. Experience shows also that in such bonds, the burlap shows very little resistance to tearing.

As concerns this difficulty, an important feature of my invention is that it affords an 35 entirely different character of adhesive bond between the burlap and the linoleum composition, paint, etc. More particularly, my invention provides for an intermediate flexible, slideable bond in the form of a film coating 40 on the threads of the fabric. This coating is preferably asphalt or other material of the type that never really becomes solid, in the ordinary sense of the word. That is to say, while it may become very fluid when 45 highly heated and may have a fairly definite solidifying point below which it becomes progressively stiffer, it retains characteristics of a super-cooled liquid at all normal temperatures. One surface of such a film adheres 50 tightly to the jute and the other to the paint or the linoleum composition, while the intervening material of the film can slowly flow to permit a sort of lubricated slip under stress, thereby permitting considerable readjustment between fibers of the threads and 55 between the thread and the linoleum or paint, without the brittle rupture effects observed in prior products. The fact that the external adhesion is greater than the internal cohesion is proved by the fact that when the burlap threads are forcibly stripped out of their bed grooves in the composition, the one 60 face of the asphalt film remains as lining in the groove while the other remains on the 65 surface of the jute thread. This indicates

how the jute and linoleum can slip endwise without the rupture of bonds or the fibers.

Furthermore, my invention provides a truly remarkable increase in resistance to tearing which seems to be due partly to the fact that by my method the asphalt is applied in such a way as to practically double the tensile strength of the jute yarn or threads, and still further due to the fact that under tearing stress the fibers do not tear one at a time in their seats, but slip out and squeeze together under the tearing twist so that the rupturing stress cannot be applied until there are several of the threads affording united resistance thereto.

As my invention affords a double remedy separately affecting each of the above described defects, it is naturally difficult to describe the invention in such a way as to clearly discriminate between the essentials necessary for a cure of one as distinguished from those necessary for cure of another. It is probable, however, that the preferred practice of the invention which is best for one is also best for the other.

As concerns warping, convexing, etc., a fundamental cause of success of my invention is final abandonment of the old idea that this defect must be cured or can be cured by waterproofing the under surface of the linoleum and shifting to the idea of an improved preliminary treatment for the burlap or other fabric. My preferred method best calculated to serve all the above enumerated functions involves treating the burlap with asphalt of such quality and under such conditions that the substance of every fiber will be materially impregnated with the asphalt, the surface of every fiber will be coated with asphalt and the thread or yarn as a whole will be saturated with asphalt, yet the open mesh spaces characteristic of the burlap and which serve a very useful function, will remain open and unclogged by the asphalt. Preferably, the warp threads are somewhat stretched, the fabric is rolled down to comparative uniformity in thickness and the crossing points of the loose weave are stuck together so that they become regularized and practically fixed, while flexibility of the fabric as a whole is preserved with only such modification as is desirable for easier handling of the fabric in the machine.

If the thus treated burlap is examined after it has cooled to normal temperatures, the physical qualities and possibilities above ascribed to it will be found more or less self-evident.

This fabric may be brought to the rolls for applying the linoleum, either hot from the squeezing rolls of the asphalt bath or if pre-cooled, it will be re-heated by the rolls of the linoleum machines. The linoleum machine may apply the linoleum composition and complete the product according to any of the

approved methods, the most usual of which are (a) rolling the linoleum composition into intimate interlocking engagement with the burlap, or, (b) pre-forming the lineoleum layer in sheeting rolls and then cementing

5 it to the fabric. In the case of pre-formed sheets as also in the case of block inlaid linoleum, made from pre-formed blocks of the composition, the asphalted fabric may be provided with a preliminary backing coat 10 of paint substantially filling the mesh and with a sticky coat closing in and bonding the fabric on the upper side. The sticky coat is of a type particularly adapted for molecular adhesion to the asphalted burlap and to 15 the sheets or blocks of linoleum composition that are pressed thereon.

The above and other features of my invention may be more fully understood from the 20 following description in connection with the accompanying drawings, in which the figures are all magnified diagrammatic views indicating as nearly as may be, matters which are not really susceptible of accurate showing 25 in black and white.

Fig. 1 is a detail face view indicating something of the weave and irregularities of burlap.

Figure 2 is a similar view of the saturated 30 burlap.

Fig. 3 is a face view of a fragment of linoleum with the surface layer broken away to show the saturated burlap with the composition interlocked with the meshes thereof.

Fig. 4 is a section on the line 4—4, Fig. 3.

Fig. 5 is a sectional detail showing the asphalted fabric of Fig. 2 with backing paint applied thereto.

Fig. 6 is a similar view showing the fabric 40 and backing paint of Fig. 5 with the sticky coat and linoleum composition applied to complete the article.

As shown in Fig. 1, the fabric may be of very primitive form, comprising slightly or 45 irregularly twisted threads or yarns of various sizes, the warp threads at 1, being square woven alternately under and over the weft threads 2, in such loose mesh as to leave ample openings 3 through the fabric. When 50 treated with very hot liquid asphalt as described below, the fabric will have its fibers blackened, compressed and flattened, as indicated more or less unsuccessfully in Figs. 2 and 3.

A preferred method is to take jute burlap, run it under submerging rolls in a hot asphalt bath to thoroughly impregnate the threads, and subsequently to remove a portion of the absorbed asphalt, particularly that 55 which is mechanically held, by means of the drawing rolls at the end of the bath which serve to squeeze the impregnated fabric. This squeezing operation I have found most advantageous in accomplishing that particular 60 aim of my invention, namely, to thoroughly

impregnate or coat the individual threads of the burlap with the waterproofing asphalt while avoiding any substantial accumulation or retention of asphalt in the normally open meshes of such burlap.

The asphalt may be about half and half natural asphalt and petroleum asphalt and the mixture will have a definable melting point which may be taken as somewhere around 150° F., but there are many different standards of what constitutes melting of asphalt, and my range of melting points might be given from as low as 135° F. up to as high as 175° F. For present purposes, it is sufficient to note first, that the melting point is substantially above the highest natural or climate temperatures and substantially below the boiling point of water. Another important feature is that the asphalt in the bath is maintained at far higher temperatures, say, 400° F., as a desired standard with, say, 350° F. to 450° F. as range of variation. At these high temperatures, the asphalt is very thin and readily saturates the jute and in fact would burn and weaken 70 the fiber of the jute if allowed to do so. I have discovered, however, that there is enough free moisture naturally present in the jute to protect it for a short time and that the asphalt is so fluid that impregnation of 75 the fibers and saturation of the yarn can be completed before any real harm results. Boiling off of such water absorbs latent heat and prevents rise of temperature in the jute as long as it is present in sufficient quantities. I have found that enough of the water 80 can be boiled off and the jute fibers impregnated and the yarn saturated as above described by asphalt maintained at 400° F. by drawing the fabric through the bath at a 85 rate of, say, 150 feet per minute through a submerged path of, say, 50 feet, thereby exposing it to the heat and saturating action of the asphalt for a period of, say, 20 seconds. Another feature of the saturation is the 90 squeezing out of excess asphalt by powerful rolls, like calendering rolls, at the end of the bath. In these rolls the individual yarns are squeezed too dry but this is compensated for by excess asphalt trapped in the 95 interspaces or meshes and sucked back into the yarn when the latter expands after release from pressure of the rolls.

In the above illustrative examples, various burlaps have been found to take up 100 asphalt to the extent of, say, 60% to 90% of the weight of the burlap, but from my previous description of the functions to be served by the asphalt, it will be evident that wide variations in the method are possible; 105 as also in the percentages, temperatures, distances, speeds, and materials.

In Figs. 3 and 4, I have shown a completed linoleum made by rolling on and into the 110 fabric 1, 2, composition, 4, the pressure being 115

such that portions 4a of the composition are compressed into the mesh spaces, 3. These portions 4a are mechanically interlocked with the threads, 1, 2, as well as being in 5 molecular or adhesive engagement therewith through the medium of the thin films of yieldable asphalt. They also serve the mechanical function of relatively solid filling blocks preventing distortion or skewing of 10 the threads of the fabric.

Though my invention makes it unnecessary 15 I may improve the appearance of the under or floor face of the linoleum shown in Figs 3 and 4 by giving it a coat of paint as indicated at 5.

In Figs. 5 and 6 I have shown block inlaid linoleum made in accordance with my invention. In this case paint, 5, is first applied with portions 5a flowed or forced to fill the 20 mesh openings, 3, and into interlocking engagement with the threads 1. When this has set the sticky coat 6 is applied and onto this are pressed the pre-formed linoleum blocks 4, 4a.

25 Linoleum made as above is tougher and will resist tearing far better than any before known; it will roll to a much smaller diameter without damage, and will even stand quite sharp flexing without breaking. If 30 fixed, until the linoleum composition breaks, it crumbles little or not at all and when bent flat again will usually appear unbroken and may be even self-healing to some extent where high grade linoleum composition is used. It will not convex or warp on the floor 35 but, on the contrary, will actually flatten itself to the floor when forcibly bent away. It is obvious that these results are not due to any mechanical constraint imposed by the 40 weight of the asphalt for the amount is far too small and there is every reason to believe that it is due to the semi-fluid nature of the bonding film that unites the fabric to the 45 composition and to the complete exclusion of moisture from the fabric. My invention clearly demonstrates that exclusion of moisture from the lower or floor face of the linoleum is unnecessary and to my mind it further demonstrates that the bonding film of 50 asphalt does exercise a semi-fluid or quasi-lubricating function sufficient to afford minute slip or yield of the bonded fibers without breaking or impairing the bond.

55 As will be evident from the foregoing, my invention applies to linoleum-like products even where modern equivalents or substitutes are used, as for instance, various oils, or oxidized or polymerized oils or pitches used in place of the linseed product; also in 60 place of the asphalt various other bituminous products or oils or pitches may be used to serve some or all of the desired functions; and some of these may be served where the fabric is treated with the asphalt or equivalent, regardless of whether it is a coating, or

is a saturation, or is an impregnation of the material of the fiber, any one or two, or all three being new and useful for some or all of the above purposes.

I claim:

1. The method of making linoleum, which includes first waterproofing the individual threads or yarns in open-mesh fabric, while preventing any substantial retention of the waterproofing material in the normally open meshes, and then associating the fabric with 70 the linoleum composition.

2. The process of making linoleum, which includes first waterproofing the individual threads or yarns in open-mesh fabric by submerging the fabric in asphalt maintained at a temperature far above the boiling point of water for a brief period, then removing the excess of asphalt beyond that required to impregnate and coat the threads of the fabric, 80 and preventing the retention of any substantial amount of asphalt in the normally open meshes, and then associating the fabric with 85 the linoleum composition.

3. The process of making linoleum, which includes first waterproofing the individual threads or yarns in open-mesh fabric by submerging the fabric in asphalt having a melting point between approximately 135° F. and 175° F., then removing the excess of asphalt 90 beyond that required to impregnate and coat the threads of the fabric, and preventing the retention of any substantial amount of asphalt in the normally open-meshes, and then associating the fabric with the linoleum composition.

4. The method of making linoleum, which includes first submerging open-mesh fabric in asphalt maintained at a temperature far above the boiling point of water for a brief 100 period, then passing the fabric between pressure rolls operating to squeeze the threads of the fabric to an over dry condition, restoring a desired amount of the asphalt by absorption of the excess asphalt that is trapped in 105 the unsqueezable mesh openings in the fabric, and finally associating the fabric with the linoleum composition by any of the known or approved methods.

5. The method of making linoleum, which includes first submerging open-mesh fabric in asphalt maintained at a temperature far above the boiling point of water for a brief period, then passing the fabric between pressure rolls operating to squeeze the threads of the fabric to an over dry condition, restoring a desired amount of the asphalt by absorption of the excess asphalt that is trapped in 110 the unsqueezable mesh openings in the fabric, and finally associating the fabric with the linoleum composition by forcing the linoleum composition into intimate interlocking engagement in the meshes of the fabric.

6. The method of making linoleum, which includes first saturating open-mesh fabric 115

with asphalt, having a normal melting point of about 150° F., maintained at a temperature above 350° F., then passing the fabric between pressure rolls operating to squeeze <sup>5</sup> the threads of the fabric to an over dry condition, restoring a desired amount of the asphalt by absorption of the excess asphalt that is trapped in the unsqueezable mesh openings in the fabric and finally associating the fabric <sup>10</sup> with the linoleum composition.

7. A floor covering comprising a wearing surface of linoleum-like composition and an open mesh backing fabric, the individual threads of said fabric being impregnated <sup>15</sup> with a semi-solid adhesive waterproofing material, and the mesh openings of said fabric being substantially devoid of said waterproofing material.

8. A floor covering comprising a wearing <sup>20</sup> surface of linoleum-like composition and an open mesh backing fabric, the individual threads of such fabric being impregnated with asphalt and the mesh openings of said fabric being substantially devoid of asphalt.

9. A floor covering comprising a wearing surface of linoleum-like composition, and an open mesh backing fabric embedded therein and bonded thereto through the medium of thin films of a semi-solid adhesive waterproofing material the individual threads of <sup>25</sup> the fabric being impregnated with said waterproofing material and the mesh openings of the fabric being substantially devoid of said waterproofing material.

10. A floor covering comprising a wearing surface of linoleum-like composition, and a backing of open mesh fabric, the individual threads of the fabric being impregnated with asphalt and the mesh openings of the fabric <sup>30</sup> being substantially devoid of asphalt, the linoleum-like composition extending into the mesh openings of the fabric between the asphalt impregnated threads and forming a mechanical interlock with said fabric.

45 In testimony whereof, I affix my signature.  
MERLE S. MC CONOUGHEY.